

1

2,786,734

**PROCESS OF FIXING MECHANICAL FINISHES TO  
CELLULOSE FABRICS BY APPLYING ISOCYANATE-BISULPHITE ADDITION SALTS**

John Gwynant Evans, Menston-in-Wharfedale, James Harry Leach, Morley, Leeds, and William Salkeld Meals, Bradford, England, assignors to The Bradford Dyers' Association Limited, Bradford, England, a company of Great Britain

No Drawing. Application March 2, 1951,  
Serial No. 213,691

Claims priority, application Great Britain March 10, 1950

**2 Claims. (Cl. 8—116.2)**

This invention relates to the treatment of cellulosic materials whereby they are given an enhanced resistance to water or steam of effects produced mechanically on such materials. By "cellulosic materials" we mean cellulosic films, foils, paper and pulp, yarns, fibres and woven or non-woven, e. g. knitted, felted or bonded-web, fabrics of natural or regenerated cellulose, cellulose esters or ethers or their mixtures with other fibres. In the case of certain finishing effects, e. g. embossing and moire, the invention is also applicable to fabrics composed wholly or mainly of natural silk, and such fabrics are included by the term "cellulosic materials."

The mechanical finishes which come into consideration include, for example, pressing, calendering, schreinering, embossing, beetling, rippling, the special finishes known as moire and cire, and mechanically enforced dimensional adjustment such as hereinafter described. Other finishes include the crimping and polishing of yarns, and the finish obtained by folding a fabric and pressing so as to form pleats. Normally these finishes are very sensitive to moisture and they may be substantially diminished or even destroyed by water or by steam pressing processes such as are common in the final stages of garment manufacture or by laundering. It is the object of the present invention to provide a process which will substantially overcome such disadvantage.

In a co-pending application Serial No. 200,312, filed December 11, 1950, now abandoned, we have described the use of aliphatic and aromatic isocyanates and isothiocyanates applied from aqueous emulsion to textiles, followed by drying and mechanical treatment with or without a subsequent heat treatment as a means of producing mechanical finishes of much improved resistance to laundering and to the influence of moisture generally.

We have now discovered that the reaction products of bisulphites with mono- or poly-functional isocyanates and isothiocyanates (hereinafter termed "isocyanate-bisulphite reaction products") may be very advantageously used in a similar manner to produce moisture- and wash-resistant mechanical finishes on cellulosic materials. Except in the specific examples, the term "isocyanate" will be used hereafter to include "isothiocyanate." The term "chalcogen" having an atomic weight not exceeding that of sulphur, covers oxygen and sulphur only in accordance with accepted terminology.

This discovery is all the more unexpected since we have evidence that the nature of the reaction when the isocyanate-bisulphite reaction products are applied to cellulosic materials and heated is different from the reaction of the corresponding isocyanates themselves. This evidence is disclosed in our co-pending application Serial No. 213,692, filed March 2, 1951, relating to the modification of properties of cellulosic materials by the appli-

2

cation of these isocyanate-bisulphite reaction products. Therein it is described, inter alia, that, whereas the application of an isocyanate to a cellulosic material followed by heating, results in a decreased affinity for direct dyes, the application of the corresponding isocyanate-bisulphite reaction product under similar conditions has a diametrically opposite effect and increases the affinity for direct dyes.

The process according to the present invention comprises incorporating in a cellulosic material an isocyanate-bisulphite reaction product, applying the effect or finish thereto and submitting it to heat. The preferred method is to impregnate the materials with an aqueous solution or dispersion of the isocyanate-bisulphite reaction product, dry or partially dry the material, then apply the effect or finish and submit the material to heat. It will be understood that, when applying the said reaction product in an aqueous medium, the mechanical finish must be applied afterwards, since it would otherwise be impaired by the aqueous medium.

The optimum temperature for the heat treatment is the decomposition temperature of the isocyanate-bisulphite reaction product used. The heat treatment will normally be of 3-15 minutes' duration at a temperature of 100° C. to 200° C., but if a lower temperature is used the time necessary will be substantially greater. It may be possible, in some cases, to carry out the mechanical finishing treatment and the heat treatment simultaneously. The heat treatment may be carried out by any of the conventional methods, but preferably is effected between 125° C. and 180° C. for a few minutes in stenters or hot air chambers or through machines which use infra-red radiation as the source of heat. Alternatively this heat treatment may be effected by passing the material through a bath of molten metal, e. g. containing low temperature melting alloys, or less preferably may be effected by treating the material with steam.

One method of making the isocyanate-bisulphite reaction products is to disperse the isocyanate in a saturated aqueous solution of an alkali metal bisulphite, e. g. sodium bisulphite, preferably in about equimolecular proportions, from which after a short time the isocyanate-bisulphite reaction product will separate out. Liquid isocyanates may be stirred into the saturated bisulphite solution but solid isocyanates should be dissolved in an organic solvent such as benzene, toluene or xylene first.

The isocyanate-bisulphite reaction products may be dried at relatively low temperatures to white odourless solids. They are in many cases soluble in water to give stable solutions in contradistinction to the corresponding isocyanates which are decomposed by water. The sodium compounds of isocyanate-bisulphite reaction products are generally soluble in water, but the corresponding potassium salts are not so readily soluble in water. Where the solubility of the salts is low they can be used in aqueous dispersion. Conditions of use which lead to the hydrolysis of the reaction products, e. g. heating of aqueous solution, should be avoided.

Alternatively to, but less preferably than, the application of the isocyanate-bisulphite reaction product itself to the material, this product can be produced in situ either by the application of the isocyanate first followed by the bisulphite, or vice-versa, in both cases with a final heat treatment as already described. Thus the isocyanate may be applied to the material from a solution in an organic solvent which is then evaporated whereafter the bisulphite is applied from aqueous solution, and the cellulosic material dried and heat treated. Similarly the bisulphite can be applied to the material first from an

aqueous solution followed by drying and the application of the isocyanate from an organic solvent solution, the solvent is evaporated and the heat treatment carried out.

A further modification of the invention includes the emulsification of the isocyanate in a dilute aqueous bisulphite solution and the application of this emulsion to the cellulosic material, followed by drying and heating. In dilute solutions of bisulphites the reaction does not readily take place but on drying and concentrating on the fabric the isocyanate-bisulphite reaction can be carried out.

Although mono-functional isocyanates may be used to react with the bisulphite, it is preferable to use poly-functional isocyanates such as a di- or tri-isocyanate. In the case of the aromatic isocyanates, the tri-functional are preferred to the di-functional, whilst, in the case of the aliphatic isocyanates, it is preferred to use the di-functional having an aliphatic chain of not more than 10 carbon atoms. If mono-functional isocyanates are to be used, it is preferable that they be either aromatic isocyanates or aliphatic isocyanates with a chain containing not more than 8 carbon atoms. The isocyanates and isothiocyanates which are employed in accordance with the present invention are monomeric compounds of the formula  $R.(N:CX)_n$  where X is a chalcogen having an atomic weight not exceeding that of sulphur, n is a whole number not exceeding 3, and R represents monomeric aromatic and aliphatic hydrocarbon radicals, the aromatic radicals having monocyclic aryl hydrocarbon groups of not more than seven carbon atoms and the aliphatic hydrocarbon radicals having a chain of not exceeding ten carbon atoms and when n is 1, contain not more than eight carbon atoms. The bisulphite reaction products are addition salts having the formula  $R.(NH.CX.SO_3M)_n$  where X, n and R are as defined above, and M is an alkali metal.

Specific examples of suitable isocyanate-bisulphite reaction products are the bisulphite reaction products of phenyl isocyanate, hexamethylene di-isocyanate, m-toluylene di-isocyanate, m-phenylene di-isocyanate, the mixture of poly-isocyanates in xylene solution under the registered trademark Vulcafor V. C. C., and any of the corresponding isothiocyanates, and also allyl isothiocyanate. Further examples include the bisulphite reaction products of toluene 2:4 di-isocyanate, toluene 2:4:6 tri-isocyanate, mixtures of toluene 2:4 and 2:6 di-isocyanates and methylene bis-p-phenylene isocyanates.

We have found that the heat treatment may also be advantageously effected in the presence of an amide, an amidine or an amino-triazine. These are preferably added to the aqueous solution of the isocyanate-bisulphite reaction product and the process carried out as already described.

Suitable amides are urea, thiourea, acetamide, sulphonamide or p-toluene sulphonamide and dicyandiamide; suitable amidines include guanidine and amino guanidine, and suitable amino triazines include melamine.

The improvement which is brought about by these amides, amidines or amino triazines is demonstrated by the firmer handle of the finished fabric and the greater resistance of the finished effect to washing.

It will be clear that by local application of the bisulphite compounds as by printing or stencilling it is possible to get patterned effects on washing in which the mechanical finish has been fixed locally. Alternatively, the isocyanate-bisulphite reaction product may be applied all over the fabric but be rendered locally ineffective by the prior local application to the fabric of chemical resists, e. g. strongly alkaline pastes, or be prevented from reaching certain portions of the fabric by the prior application of mechanical resists, e. g. waxes to such portions. As a further alternative, discharge methods may be used, e. g. by applying the isocyanate-bisulphite reaction product all over the fabric and then, prior to the heat treatment, applying a pattern of a strongly alkaline paste.

The present invention may often be used with advantage in conjunction with the above-mentioned dye process described in our co-pending application Serial No. 213,692. For example, a dye may be included in the solution of the isocyanate-bisulphite reaction product before applying same to the material to be treated, thereafter effecting the mechanical finishing treatment. Alternatively dye may be applied after the mechanical finishing treatment and after the subsequent heat treatment.

Apart from water solubility and the stability of their aqueous solutions a great advantage of the isocyanate-bisulphite reaction products as compared with the corresponding isocyanates is the pleasanter and more efficient operating conditions. Many of the isocyanates are volatile during drying and heating and their fumes have, in a number of cases, pronounced physiological effects. The isocyanate-bisulphite reaction products give rise to no fumes, thus avoiding unpleasant effects on the operatives and, since the whole of the agent applied to the textile is used and not lost as vapour, the process is more efficient.

It has been found that the present invention may very suitably be used in the case where the mechanical finish is designed to alter forcibly the dimensions of a fabric.

For example, a well known method for producing a dimensionally-adjusted woven fabric is to pass the fabric through a machine which forcibly reduces the dimensions of the fabric by pressing the yarns closer together, or, if so desired, which forcibly increases the dimensions of the fabric by pulling the yarns further apart. Such machines are described in British specifications No. 359,759 and No. 372,803.

The invention is applicable to fabrics that have already been finished in a conventional manner, that is to say the treatment may be applied for example to fabrics which contain softening agents, lubricating agents, antiseptics or which have been antcreased or stabilised by means of thermosetting resinous condensates.

The invention may also be applied by treating fabrics with the isocyanate-bisulphite reaction products before or simultaneously with conventional finishing agents.

In the following examples which illustrate the invention the parts are by weight.

#### Example I

84 parts of hexamethylene di-isocyanate are added to 310 parts of a solution of sodium bisulphite in water containing 104 parts of sodium bisulphite. The two liquids are intimately mixed by means of vigorous agitation, and as the reaction proceeds a white crystalline solid separates. The mix eventually becomes a stiff paste, from which the bisulphite compound can be obtained by filtration and washing with acetone, followed by drying at 50-60° C.

A plain cotton fabric is impregnated in a solution prepared by dissolving 7.5 parts of the compound prepared as above in 92.5 parts of water. The fabric after mangleing is partially dried so that it retains 15% of moisture, and glazed by passage between a heated metal cylinder at 200° C., and a compressed paper bowl. The glazed fabric is now heated to 150° C. for 10 mins.

The glaze imparted to the fabric is now resistant to repeated washing in aqueous soap solutions at 75° C.

#### Example II

A mercerised cotton fabric is impregnated in a solution containing 10 parts of hexamethylene di-isocyanate bisulphite compound prepared as in Example I, in 90 parts of water, mangled and dried at open width on a stenter. The dry fabric is steam moistened, and cire embossed by passage between a heated engraved metal cylinder at 180° C., and a compressed paper bowl. The embossed fabric is then heated to 150° C. for 10 minutes. The embossed pattern is now resistant to repeated washing in soap.

*Example III*

A plain cotton fabric is printed through a silk screen with a thickened paste made as follows:

5 parts of the bisulphite compound of hexamethylene di-isocyanate, prepared as in Example I, is dissolved in 45 parts of water and this solution is stirred into a dispersion of 4 parts of locust bean gum in 46 parts of water.

The printed fabric is dried, and steamed so that it contains 15% moisture, and glazed by passage between a heated metal cylinder at 180° C., and a compressed paper bowl. The fabric is then washed in aqueous soap solution at 60° C., when the glaze in the unprinted parts is removed, whereas that in the printed parts is retained. In this way a localized glazed effect is produced which is resistant to laundering.

*Example IV*

A cotton fabric is impregnated in a solution containing 4 parts of dicyandiamide and 6 parts of the bisulphite compound of hexamethylene di-isocyanate, prepared as in Example I, in 90 parts of water. After impregnation the fabric is partially dried until it contains 15% of moisture, and is then glazed in known manner on a calender at 200° C.

The glazed fabric is then subjected to a heat treatment at 150° C. for 10 minutes. The incorporation of dicyandiamide results in a much firmer handle of the glazed fabric, the characteristics of which are resistant to repeated laundering.

*Example V*

A plain cotton fabric is printed as in Example III. The steamed, dried fabric is glazed in known manner on a calender at 190° C., and heated at 150° C. for 10 minutes. The glazed fabric is then passed into a dyebath at 90° C. containing 0.5 gm. per litre Polar Brilliant Red G (Geigy Colour Company) (New Colour Index "Acid Red No. 122") and 5.0 gms. per litre sodium sulphate, with a volume ratio of 40:1. In this way, the fabric is dyed in the printed parts which at the same time retain their lustre, the unprinted parts lose their lustre in the hot dyebath, and are not dyed. In this way a coloured localized glazed fabric is produced fast to washing.

*Example VI*

A plain cotton fabric is printed through a silk screen with a thickened paste made in the following manner:

5 parts of the bisulphite compound of hexamethylene di-isocyanate prepared as in Example I are dissolved in 20 parts of water and stirred into 30 parts of a dispersion containing 3 parts of locust bean gum. 2 parts of Polar Brilliant Red G are dissolved in 40 parts of water and this solution is stirred into the paste.

The printed fabric is dried, and steam moistened, glazed on a calender at 190° C. in known manner, followed by heating at 150° C. for 10 minutes. The glazed fabric is then secured in dilute aqueous soap solution at 40° C. for 10 minutes when the glaze in the unprinted parts is removed. Thus a coloured printed glazed effect is produced which will withstand soaping at 70° C.

*Example VII*

A plain cotton fabric is impregnated in a solution containing 10 parts of hexamethylene di-isocyanate in 90 parts of benzene, and dried to remove the solvent at 60° C. The fabric is then padded through a solution containing 15 parts of sodium bisulphite in 85 parts of water. After mangling the fabric is maintained in the wet condition for 2 hours during which time the reaction between the isocyanate and the sodium bisulphite proceeds.

The fabric is then partially dried, so that it retains 15% of moisture, and embossed by passage between a heated engraved metal cylinder at 150° C., and a superelastic cotton bowl. The embossed fabric is then heated to

150° C., for 10 minutes, followed by rinsing in water at 45° C. The embossed design on the fabric is resistant to washing at 70° C. in dilute aqueous soap solutions.

*Example VIII*

5 The potassium bisulphite reaction product of hexamethylene di-isocyanate is prepared by first reacting hexamethylene di-isocyanate and sodium bisulphite solution as described in Example I. The paste so obtained is dissolved in 310 parts of water and the solution is heated to 60° C. with the addition of 84 parts of potassium chloride and filtered to remove impurities. On cooling to 5° C. crystals of the more sparingly soluble potassium salt are obtained.

10 15 A plain cotton fabric is impregnated in a solution containing 10 parts of the potassium bisulphite compound of hexamethylene di-isocyanate and 5 parts of urea in 85 parts of water. The fabric is dried so that it contains approximately 15% of moisture and is then embossed by passage between an engraved metal cylinder at 180° C. and a compressed paper bowl. The fabric is heated at 145° C. for 10 minutes. The embossed design is now resistant to repeated washing in soap solution.

*Example IX*

25 30 parts of metatoluylene di-isocyanate are mixed with 130 gms. of sodium bisulphite solution, 100 gms. of which contain 30 gms. of sodium bisulphite. The two liquids are intimately mixed by means of vigorous agitation, and after 2 hours the mix becomes a stiff paste. The solid precipitate is filtered, washed and dried at 60° C.

30 35 A cotton fabric incorporating a woven design is impregnated in a solution of 5 parts of the bisulphite reaction product with meta tolulylene di-isocyanate in 95 parts of water and dried. The dry fabric is steam moistened, and friction glazed by passing between a heated metal cylinder at 180° C., and a compressed paper bowl. The glazed fabric is then heated at 145° C. for 10 minutes. The glazed effect is now resistant to repeated washing in soap solutions and the woven design is considerably enhanced in appearance.

*Example X*

45 50 A pure silk fabric is impregnated in a solution of 10 parts of the reaction product of hexamethylene diisocyanate and sodium bisulphite (prepared as in Example I), and 10 parts of urea in 80 parts of water. After drying the fabric is steam moistened and passed in double thickness between a heated metal cylinder at 70° C., and a compressed paper bowl to produce a moire effect. The fabric is then heated for 4 minutes at 150° C. The moire effect is now resistant to repeated treatments in soap solutions.

*Example XI*

55 60 A warp twill viscose rayon staple-fibre fabric is impregnated in a solution containing 10 parts of hexamethylene di-isocyanate bisulphite compound, prepared as in Example I, in 90 parts of water, mangled and dried. The fabric is then compressively shrunk by treatment as described in British Patent No. 372,803 and heated at 150° C. for 10 minutes. The effect of this treatment is illustrated in the following table showing the amount of shrinkage obtained by washing the fabric in a liquor containing 0.25 part of soap per 100 parts of aqueous solution.

|    |                                                                                                                                                | Warp shrinkage, percent | Weft shrinkage, percent |
|----|------------------------------------------------------------------------------------------------------------------------------------------------|-------------------------|-------------------------|
| 70 | 1. Untreated fabric                                                                                                                            | 14.0                    | 2.5                     |
|    | 2. As 1, compressively shrunk according to B. P. 372,803                                                                                       | 6.4                     | 1.0                     |
| 65 | 3. Fabric impregnated in sodium bisulphite compound of hexamethylene di-isocyanate, compressively shrunk according to B. P. 372,803 and heated | 2.1                     | 0.6                     |

## Example XII

A viscose rayon staple-fibre yarn is impregnated with a solution of 10 parts of the sodium bisulphite reaction product of hexamethylene di-isocyanate and 5 parts of urea in 85 parts of water. The yarn is partially dried to a moisture content of 15%, deformed by crimping, and then heated at 145° C. for 10 minutes. The crimp is rendered durable to repeated soaping.

What we claim is:

1. Process for improving the resistance to water and aqueous treatments of effects produced by mechanical treatment on cellulose textiles comprising impregnating such material with a bisulphite addition salt having the formula  $R.(NH.CX.SO_3M)_n$  where X is a chalcogen having an atomic weight not exceeding that of sulphur, n is a whole number not exceeding 3, M is an alkali metal, and R represents monomeric aromatic and aliphatic hydrocarbon radicals, the aromatic radicals having monocyclic groups of not more than seven carbon atoms and the aliphatic hydrocarbon radicals having a chain not exceeding ten carbon atoms, and when n is 1 not more than eight carbon atoms, applying the mechanical treatment to produce the desired effect, and submitting the material to heat at a temperature at least as high as the decomposition temperature of the addition product but below that of any deleterious effect on the impregnated material, in which process there is also applied to the material a compound selected from the group consisting of urea, thiourea, dicyandiamide, p-toluene sulphonamide, guanidine, amino-guanidine and melamine, so that said compound is present in the material during the heat treatment.

2. Process for improving the resistance to water and aqueous treatments of effects produced by mechanical treatment on cellulose textiles comprising impregnating such material with a bisulphite addition salt having the formula  $R.(NH.CX.SO_3M)_n$  where X is a chalcogen having an atomic weight not exceeding that of sulphur, n is a whole number not exceeding 3, M is an alkali metal, and R represents monomeric aromatic and aliphatic hy-

drocarbon radicals, the aromatic radicals having monocyclic groups of not more than seven carbon atoms and the aliphatic hydrocarbon radicals having a chain not exceeding ten carbon atoms, and when n is 1 not more than eight carbon atoms, applying the mechanical treatment to produce the desired effect, and submitting the material to heat at a temperature at least as high as the decomposition temperature of the addition product but below that of any deleterious effect on the impregnated material, in which process the impregnation is with an aqueous medium containing the addition salt and the impregnated material is at least partially dried prior to application of the mechanical treatment, and in which the aqueous medium includes a compound selected from the group consisting of urea, thiourea, dicyandiamide, p-toluene sulphonamide, guanidine, amino-guanidine and melamine, so that said compound is present in the material during the heat treatment.

## References Cited in the file of this patent

## UNITED STATES PATENTS

|           |                |               |
|-----------|----------------|---------------|
| 2,121,005 | Bener          | June 21, 1938 |
| 2,121,006 | Bener          | June 21, 1938 |
| 2,123,153 | Rivat          | July 5, 1938  |
| 2,217,696 | Milburn        | Oct. 15, 1940 |
| 2,284,895 | Hanford        | June 2, 1942  |
| 2,339,913 | Hanford        | Jan. 25, 1944 |
| 2,370,405 | Kaase          | Feb. 27, 1945 |
| 2,468,716 | Nyquist et al. | Apr. 26, 1949 |
| 2,643,958 | Kleiner et al. | June 30, 1953 |
| 2,710,816 | Evans et al.   | June 14, 1955 |

## FOREIGN PATENTS

|         |               |              |
|---------|---------------|--------------|
| 521,116 | Great Britain | May 13, 1940 |
|---------|---------------|--------------|

## OTHER REFERENCES

Chemical Abstracts, vol. 44, January 1950, pages 115-116.